

C. THOM, R. W. DIAMOND AND S. G. BLAYLOCK.  
PROCESS FOR THE MAGNETIC SEPARATION OF ORES.  
APPLICATION FILED APR. 30, 1920. RENEWED OCT. 14, 1921.

1,398,051.

Patented Nov. 22, 1921.

Flow Sheet For Magnetic Separation of Ores.



Inventors

Clarence Thom  
Ralph W. Diamond  
Silvyn G. Blaylock  
Per Thors & Knudsen  
attorneys.

# UNITED STATES PATENT OFFICE.

CLARENCE THOM, RALPH WILLIAM DIAMOND, AND SELWYN GWILLYM BLAYLOCK,  
OF TRAIL, BRITISH COLUMBIA, CANADA, ASSIGNORS TO THE CONSOLIDATED MIN-  
ING & SMELTING COMPANY OF CANADA, LIMITED, OF MONTREAL, QUEBEC,  
CANADA.

## PROCESS FOR THE MAGNETIC SEPARATION OF ORES.

1,398,051.

Specification of Letters Patent.

Patented Nov. 22, 1921.

Application filed April 30, 1920, Serial No. 377,929. Renewed October 14, 1921. Serial No. 507,774.

To all whom it may concern:

Be it known that we, CLARENCE THOM, a citizen of the United States, and RALPH WILLIAM DIAMOND and SELWYN GWILLYM BLAYLOCK, British subjects, residents of the city of Trail, in the District of Kootenay and Province of British Columbia, Dominion of Canada, have invented a new and useful Process for the Magnetic Separation of Ores; and we hereby declare the following to be a full, clear, and exact description of the same.

Our invention relates to a process by which some sulfid ores may be made highly susceptible to magnetic influence for the magnetic separation of the constituents, and involves four consecutive steps, two of which are interdependent and of the utmost importance to the success of the final operation.

The first step, is to heat the ore, without roasting, to a temperature, which when the ore is properly cooled, will yield the maximum magnetic susceptibility.

The advantage of this is, that when a sulfid ore, for example one containing free and combined iron compounds such as pyrrhotite and marmatite respectively direct from the mine, is ground fine and subjected to magnetic separation, only about 25% of the total iron content is sufficiently amenable to magnetic influence to be separated by commercial magnetic machines. When the ore is subjected to a heat of from 800° F. to 1200° F. according to its fineness and the ore is allowed to cool slowly practically 100% of the pyrrhotite is rendered sufficiently susceptible to be separated by the same magnetic machines. The best results

are obtained when the ore is heated in a coarse state—two inch pieces being easiest to handle, but pieces as large as 6 inches cubed may be heated and the cores of the pieces as well as the outer rims will be rendered magnetic without the interior becoming oxidized. An over heat of the ore, however, is detrimental to the process, and therefore it is necessary to stay within temperature limits as well as time limits, these limits being governed by the ore being treated, as ores from different mines and localities may require different temperature and time treatments. For some ores it is found

that a temperature of about 1200° F., if the ore is allowed only a few minutes exposure to the heat—enough to barely heat the larger pieces through—will give good results. If, however, the ore is exposed to this high heat for too long a time and any oxidation or even a tendency to melt the sulfid out of the ore occurs, the resulting separation of the pyrrhotite from the other minerals is poor. If too, a period of heating even at 1000° F. is continued too long, the same poor result is obtained.

Satisfactory results are obtained by exposing the ore which has been crushed to about two inch mesh to a heat of 1000° F. for about nine minutes.

The progress of the ore through the kiln being relatively rapid, it is possible for the exteriors of the lumps to attain approximately a dull red heat without the interiors of the lumps becoming heated, during the direct action of the heat treatment in the kiln, and as this thorough heating of the lumps is essential for the success of the process, sufficient time must elapse during the cooling for the heat to travel through the lump by conduction.

The second step in the process, therefore, is the slow cooling of the ore after heating. If the hot ore is suddenly cooled by immersion, very poor results are obtained. In fact, in general the magnetic susceptibility of the ore is then nearly as low by this treatment as for green ore without heating. If, however, a period of fifteen minutes is allowed to elapse before the ore is cooled to a temperature of about 400° F., there is only a slight loss in the magnetic susceptibility.

The third step in the process is wet grinding in a ball mill or by any common grinding practice.

The fourth step is the magnetic separation of the magnetic sulfids from the gangue and other minerals, this being accomplished by passing water ore pulp over commercial magnetic machines.

To explain how the process may be conveniently operated, we have shown in the diagrammatic drawing a flow sheet of an apparatus suitable for the purpose.

The ore as it is received from the mine is crushed and passed over a "screen" pref-

erably of about one fourth to three eighths inch mesh to separate the fines from the oversize.

The oversize is then delivered into a slowly revolving "brick lined kiln" set at a suitable inclination and of such dimensions that the feed progresses through it at a speed to deliver the ore at the discharge end at a dull red heat, this heat being sufficient to render the ore amenable to magnetic influence but not sufficient to roast it or cause any apparent chemical change in its constituents.

The fines, separated from the oversize, by-pass the kiln and combine with the heated ore when delivered from the discharge end of the kiln, and take up part of the heat from the oversize sufficient for the purposes of the process.

20 The whole product then passes through a revolving "cooling cylinder" of such dimensions and installation that the feed of heated ore progresses through it under such conditions of heat exchange and limitations 25 of time as to deliver the ore at the discharge end at a temperature which will result in the maximum magnetic susceptibility being attained when the ore is properly cooled.

30 The cooling may take place in either a reducing atmosphere, a neutral atmosphere, or even a slightly oxidizing atmosphere, provided the ore is heated in lumps and the cooling operation is sufficiently slow to retain the magnetic susceptibility of the ore.

To provide this atmosphere air may be blown through the cylinder counter current to the heated ore.

From the cooling cylinder, the ore goes 40 direct to the "ball mill", where it is ground sufficiently fine to separate the different mineral particles, and from the ball mill the ground ore then passes to the "electro-magnetic machines" where the minerals are 45 separated.

In a series of tests conducted to determine the value of this process for the separation of iron sulfid ores, it was ascertained that before heating only about 25% 50 of the iron content was susceptible of magnetic attraction.

After heating the ore to the temperature above specified and immediately cooling it, 46.6% of the total iron content was separated.

After heating and allowing the ore five

minutes to cool, 47.6% of the total iron content was separated.

After heating and allowing the ore ten minutes to cool, 66.8% of the total iron content was separated.

After heating and allowing the ore fifteen minutes to cool, 76.2% of the total iron content was separated.

After heating and allowing the ore twenty minutes to cool, 77.9% of the total iron content was separated.

After heating and allowing the ore to be cooled for twelve minutes by an air blast and then immersed or quenched, 80.5% of the total iron content was separated, this separation representing practically the whole of the pyrrhotite.

What we claim is:

1. A process for the magnetic separation 75 of ores which consists of heating the ore without roasting to a temperature ranging from 800° F. to 1200° F. which when the ore is properly cooled will yield the maximum susceptibility, then artificially cooling the ore under such conditions of heat exchange and time limitations ranging from five to fifteen minutes as to retain this susceptibility.

2. A process for the magnetic separation 85 of ores which consists of crushing the ore, separating the fines from the oversize, heating the latter to a temperature which will render the ore amenable to magnetic influence when properly cooled, combining the 90 fines with the oversize when heated, and cooling the ore under such conditions as to retain its magnetic susceptibility.

3. A process for the magnetic separation 95 of ores which consists of heating the ore without roasting to a temperature ranging from 800° F. to 1200° F., which when the ore is properly cooled will yield the maximum magnetic susceptibility, and then cooling the ore under such conditions of heat 100 exchange, and time limitation ranging from five to fifteen minutes as to retain this susceptibility.

Trail, B. C., March 23rd, 1920.

CLARENCE THOM.

RALPH WILLIAM DIAMOND.

SELWYN GWILLYM BLAYLOCK.

Signed, sealed and delivered in the presence of—

ANNIE MACKAY,  
CHAS. H. RICHES.